

Feb. 17, 1948.

P. H. CARDWELL ET AL

2,436,196

CHEMICAL REMOVAL OF AN ACID-SOLUBLE METAL PART IN A DEEP WELL

Filed Aug. 6, 1945



INVENTORS  
Paul H. Cardwell  
BY Louis H. Eilers

Griswold & Burdick  
ATTORNEYS

## UNITED STATES PATENT OFFICE

2,436,196

CHEMICAL REMOVAL OF AN ACID-SOLUBLE  
METAL PART IN A DEEP WELLPaul H. Cardwell and Louis H. Eilers, Tulsa,  
Okla., assignors to The Dow Chemical Company,  
Midland, Mich., a corporation of Delaware

Application August 6, 1945, Serial No. 609,252

4 Claims. (Cl. 252—8.55)

**1** The invention relates to the chemical removal of an acid-soluble metal part in a deep well. It more particularly concerns an improved method of completing wells, traversing a plurality of strata, in which a chemically soluble casing section located opposite a selected stratum is removed by chemical action to permit fluid flow between the well bore and the stratum.

In the usual well completion in which a chemically soluble section is included in the casing string opposite a productive zone, the soluble section is made of aluminum or an aluminum alloy, and its removal is effected by prolonged treatment with a quantity of hydrochloric acid.

A disadvantage of this method which limits its usefulness is that the action of the acid is quite slow, so that an inordinate amount of time is consumed in the operation and complete removal is somewhat uncertain.

A particular object of the invention is to provide an improved method of, and composition for, chemically dissolving an aluminum or aluminum alloy part, such as a casing section, in the bore of a well whereby complete rapid removal is achieved. Other objects and advantages will become apparent as the description of the invention proceeds.

According to the invention dissolution of parts or equipment made of aluminum or aluminum alloy in the well is achieved by subjecting the metal part to the corroding action of a hydrochloric acid solution to which has been added an aliphatic carboxylic acid such as acetic, amine acetic (glycine), citric, gluconic, lactic, oxalic, and tartaric. To prevent or reduce attack by the acid solution on adjacent ferrous metal parts, when such are present, an inhibitor of such action may be included in the acid solution.

The invention may be more readily understood from the following detailed description and accompanying drawing of a mode of carrying out the invention, such mode illustrating but one of various ways in which the principle of the invention may be used. In the said drawing the single figure illustrates schematically in vertical section an oil well in which an acid-soluble section located in the casing string opposite a productive zone is being removed chemically.

Referring more particularly to the drawing, the well bore 1 is provided with a casing string 2 containing an aluminum alloy (acid-soluble) sec-

**2** tion 3. Various aluminum-base alloys are suitable for the purpose as, for example, one containing about 1 per cent of silicon, about 1 per cent of magnesium, and about 0.3 per cent of chromium, the balance being aluminum. If desired, unalloyed aluminum may be used. The aluminum or aluminum alloy section is placed in the casing string so that the section is opposite a productive zone 4, the annular space between the casing string and the well hole being filled with cement 5. Such well construction is conventional and forms no part of the invention.

In preparing the well for treatment so as to remove the soluble section 3 according to the invention, the portion of the well below the productive zone 4 is bridged as with a filler 6, and a packer 7 is set in the casing at the top of the zone thereby to isolate for treatment the portion of the well containing the soluble section. The packer is provided with a central passage for admitting the outer tube 8 extending from the top of the well to just below the packer. An inner tube 9 is strung through the outer tube and extends from the top of the well to near the bottom of the soluble section.

After arranging the apparatus as described, the chemical solvent of hydrochloric acid to which has been added a suitable aliphatic carboxylic acid may be introduced through tube 9 so as to fill the space 10 in the cased portion of the well between the top of the bridge 6 and the bottom of the tube 8. As the chemical solvent becomes spent by dissolving the metal of the soluble section 3 of the casing, fresh solvent may be introduced, if necessary, thereby displacing the spent solution from the well through tube 8. It is preferable to continuously circulate the chemical solvent into the space 10 through tube 9 while the spent or partially spent solvent solution is displaced through tube 8. The amount of solvent to employ depends upon the concentration of HCl therein and the weight of the aluminum section to be removed, and may be computed on the basis of the known stoichiometrical relationship between HCl and aluminum to form aluminum chloride (AlCl<sub>3</sub>). For example, approximately 1.7 gallons of 25 per cent hydrochloric acid solution is required per pound of aluminum section. Various concentrations of HCl may be used, such as 15 to 35 per cent, concentration between about 20 and 30 per cent being preferred.

A suitable amount of one of the aforementioned aliphatic carboxylic acids to use in the hydrochloric acid solution to increase its rate of attack on the acid-soluble section is between about 0.1 and 3 per cent of the weight of the acid solution, between 0.5 and 1.0 being generally preferred.

In order to reduce or prevent attack by the acid on the ferrous metal parts of the well which may be exposed to the acid solution, particularly the steel casing adjacent to the acid-soluble part to be removed, any of the well known corrosion inhibitors may be used, such as a soluble-arsenic compound, e. g., the arsenate or arsenite of sodium, organic sulfur compounds, such as the mercaptans, organic nitrogen bases, etc., in the usual small quantities such as 0.4 to 1.0 per cent of the weight of the acid solution.

As the aluminum section of the casing dissolves, the solution becomes heated due to the liberation of heat of neutralization and hydrogen is evolved which is allowed to escape through pipe 8. The generation of heat is an advantage as it speeds the reaction.

After the aluminum section has been removed, the packer 7 and tubing strings 8 and 9 are removed so as to permit drilling out the cement sheath 11 opposite the zone 4 and removal of the bridge 6, if desired.

As illustrative of the increased rate of action of hydrochloric acid on aluminum alloy tubing brought about by the addition of a corrosion accelerator of an aliphatic carboxylic acid, tests were made in which pieces of the tubing were subjected to the dissolving action of hydrochloric acid solution to which various aluminum corrosion accelerators were added. In conducting these tests 300 cc. lots of acid were placed in a calorimeter together with a piece of an aluminum alloy containing 0.2 per cent copper, 1 per cent magnesium, 0.4 per cent silicon, 0.2 per cent chromium, the balance being aluminum, and the rate of dissolving of the aluminum alloy determined by observing from time to time the temperature attained by the reacting materials. In these tests the higher the temperature attained by the materials in a given time the faster the dissolving of the aluminum alloy occurred. Tables I and II present data so obtained.

TABLE I

Rate of reaction of 15% hydrochloric acid solution on aluminum alloy accelerated by aliphatic carboxylic acid

| Concentration and Kind of Aluminum Corrosion Accelerator | Temperature (°F.) of Reacting Materials After— |         |         |         |         |
|----------------------------------------------------------|------------------------------------------------|---------|---------|---------|---------|
|                                                          | 0 Min.                                         | 15 Min. | 30 Min. | 45 Min. | 60 Min. |
| None (Blank).....                                        | 86                                             | 106     | 121     | 135     | 149     |
| 1.0% Acetic Acid.....                                    | 86                                             | 114     | 138     | 166     | 205     |
| 1.0% Citric Acid.....                                    | 86                                             | 105     | 132     | 160     | 185     |
| 1.0% Gluconic Acid.....                                  | 86                                             | 109     | 122     | 142     | 173     |
| 0.25% Glycine.....                                       | 86                                             | 109     | 142     | 173     | 211     |
| 1.0% Glycine.....                                        | 86                                             | 108     | 127     | 150     | 173     |
| 0.25% Lactic Acid.....                                   | 86                                             | 118     | 138     | 179     | 212     |
| 0.5% Lactic Acid.....                                    | 86                                             | 117     | 152     | 210     | 214     |
| 1.0% I acetic Acid.....                                  | 86                                             | 117     | 151     | 212     | 214     |
| 3.0% I acetic Acid.....                                  | 86                                             | 108     | 122     | 134     | 148     |
| 0.25% Oxalic Acid.....                                   | 86                                             | 118     | 152     | 207     | 214     |
| 0.5% Oxalic Acid.....                                    | 86                                             | 117     | 155     | 213     | 214     |
| 1.0% Oxalic Acid.....                                    | 86                                             | 119     | 152     | 214     | 214     |
| 3.0% Oxalic Acid.....                                    | 86                                             | 112     | 156     | 175     | 212     |
| 0.10% Tartaric Acid.....                                 | 86                                             | 111     | 140     | 171     | 212     |
| 0.15% Tartaric Acid.....                                 | 86                                             | 110     | 147     | 189     | 214     |
| 0.25% Tartaric Acid.....                                 | 86                                             | 132     | 200     | 214     | 213     |
| 0.5% Tartaric Acid.....                                  | 86                                             | 125     | 158     | 214     | 214     |
| 1.0% Tartaric Acid.....                                  | 86                                             | 124     | 156     | 210     | 214     |
| 3.0% Tartaric Acid.....                                  | 86                                             | —       | 128     | 162     | 185     |

4  
TABLE II

Reaction rate of hydrochloric acid solutions on aluminum alloy accelerated by oxalic acid

| Composition of Acid Solution | Temperature (° F.) of Reacting Materials After— |        |         |         |         |
|------------------------------|-------------------------------------------------|--------|---------|---------|---------|
|                              | 0 Min.                                          | 5 Min. | 10 Min. | 15 Min. | 30 Min. |
| 20% HCl alone.....           | 86                                              | 108    | 162     | 220     | 220     |
| 20%+0.5% oxalic.....         | 86                                              | 110    | 220     | 220     | 216     |
| 20%+1.0% oxalic.....         | 86                                              | 116    | 220     | 220     | 218     |
| 25% HCl alone.....           | 86                                              | 159    | 226     | 223     | 221     |
| 25%+0.5% oxalic.....         | 86                                              | 166    | 224     | 228     | 226     |
| 25%+1.0% oxalic.....         | 86                                              | 202    | 226     | 226     | 226     |

The data in the tables show that by adding an aliphatic carboxylic acid in relatively small amount to hydrochloric acid solution its rate of attack on aluminum alloy is increased. This is evident from the fact that the temperature of the reacting materials attains a higher value in less time when an aliphatic carboxylic acid is present in the acid solution.

As a further example of the increased speed of action obtainable with our acid solution comparative tests were made in which a given weight of the acid solution was allowed to expend itself in dissolving aluminum alloy tubing, the alloy having the composition last mentioned. In these tests, it was found that whereas commercial hydrochloric acid alone containing 25 per cent by weight of HCl expended itself in about 30 minutes, the addition of from 0.5 per cent to 1 per cent of oxalic acid to the same hydrochloric acid solution increased its rate of action so that only about 20 minutes were required for its expenditure under comparable conditions. Similar tests made with 20 per cent hydrochloric acid solution gave a spending time of 45 minutes when used alone in comparison with a spending time of about 25 to 30 minutes when the same concentration of acid solution containing from 0.5 to 1 per cent of oxalic acid, respectively, was used similarly.

The term "aluminum" used herein and the appended claims is used to mean all grades of aluminum metal, and the term "aluminum alloy" means alloys of aluminum containing at least about 80 per cent of aluminum.

We claim:

1. The method of removing from a well a metal part formed of aluminum and its alloys which comprises subjecting the part to the dissolving action of an aqueous solution containing from about 20 to 30 per cent of hydrochloric acid and 0.25 to 3 per cent of oxalic acid and an inhibitor of the action of the hydrochloric acid on ferrous metal.

2. The method of removing from a well a metal part formed of aluminum and its alloys which comprises subjecting the part to the dissolving action of an aqueous solution containing from about 20 to 30 per cent of hydrochloric acid and 0.25 to 3 per cent of lactic acid and an inhibitor of the action of the hydrochloric acid on ferrous metal.

3. The method of removing from a well a metal part formed of aluminum and its alloys which comprises subjecting the part to the dissolving action of an aqueous solution containing from about 20 to 30 per cent of hydrochloric acid and 0.25 to 3 per cent of tartaric acid and an inhibitor of the action of the hydrochloric acid on ferrous metal.

4. The method of removing from a well a metal part formed of aluminum and its alloys which comprises subjecting the part to the dissolving action of an aqueous solution containing from about 15 to 35 per cent of HCl, about 0.25 to 3 per cent of an aliphatic carboxylic acid selected from the group consisting of lactic acid, oxalic acid and tartaric acid, an an inhibitor of the action of the hydrochloric acid on ferrous metal.

PAUL H. CARDWELL. 10

LOUIS H. EILERS.

REFERENCES CITED

The following references are of record in the 15 file of this patent:

UNITED STATES PATENTS

| Number    | Name           | Date          |
|-----------|----------------|---------------|
| 2,024,718 | Chamberlain I  | Dec. 17, 1935 |
| 2,128,160 | Morgan         | Aug. 23, 1938 |
| 2,140,183 | Bresler        | Dec. 13, 1938 |
| 2,175,095 | Stoesser       | Oct. 3, 1939  |
| 2,217,676 | Fry            | Oct. 15, 1940 |
| 2,232,938 | Chamberlain II | Feb. 25, 1941 |
| 2,234,790 | Zacher         | Mar. 11, 1941 |
| 2,252,973 | Hall et al.    | Aug. 19, 1941 |
| 2,261,292 | Salnikov       | Nov. 4, 1941  |
| 2,342,656 | Frye et al.    | Feb. 29, 1944 |